

# UNITED STATES PATENT OFFICE.

RUDOLF GAHL, OF MIAMI, ARIZONA, ASSIGNOR TO THE UTAH COPPER COMPANY, A CORPORATION OF NEW JERSEY,

## FLOTATION PROCESS.

1,290,166.

Specification of Letters Patent.

Patented Jan. 7, 1919.

No Drawing.

Application filed January 31, 1916. Serial No. 75,344.

To all whom it may concern:

Be it known that I, RUDOLF GAHL, a citizen of the United States, residing at Miami, in the county of Gila and State of Arizona, have invented certain new and useful Improvements in Flotation Processes, of which the following is a specification.

This invention relates to so-called "flotation processes" for the concentration of ores, and comprises a novel procedure by means of which the efficiency of these flotation processes may be very greatly improved, particularly in their application to certain ores which are unsuited for treatment by the ordinary methods. The invention will be described, in its application to the flotation of sulfid or even carbonate ores containing small percentages of copper, by means of air bubbles used in conjunction with suitable hydrocarbon substances, such as coal-tar and allied products. It is believed, however, that the present improvement is applicable to flotation processes in general, and the invention is not therefore limited to the specific conditions recited by way of example.

It is a matter of common observation that certain ores or ore-batches do not respond well to the flotation treatment; and more or less refractory ores have been discovered wherever concentration by flotation has been attempted. Even in ore bodies consisting largely of good flotation ores, portions are found which are less suited for this treatment; and in ore mixtures which respond well to flotation, portions can frequently be sorted out which do not so respond when treated by themselves. For this reason, the mixing of different ores has proven beneficial in a great many cases. In many cases, however, the ores necessary to constitute a properly responsive mixture are not available, and for such cases the process herein described will prove particularly useful.

I have observed that ores which are refractory to the ordinary flotation treatment can be handled without difficulty, and with a reasonably high degree of efficiency, provided there are added to the ore, and thoroughly mixed therewith, certain solid substances which are not themselves floated, and which do not apparently enter at all into the flotation reaction. Among such additions I

have found iron (including steel) to be particularly effective when introduced in the form of filings or other suitable state of fine subdivision. The iron may either be added in proper proportions to the feed entering the flotation machines, or it may be introduced at a previous point in the treatment, for example in the grinding apparatus.

For example, if an ore of the above-mentioned, imperfectly responsive type containing a small percentage of copper in the form of sulfid, is mixed with one-half to two per cent, or even less by weight of iron filings, together with the usual proportion of oil or equivalent material, and the whole is subjected to flotation in water or the usual flotation media, under otherwise standard conditions, air in the form of bubbles being injected or stirred into the mass, it will be found that the ore responds well to the treatment, and that excellent flotation efficiencies are obtained. The following tabular statement of actual test runs upon a small scale will serve to illustrate the results which are obtainable:

| Test No. | Grams ore. | Per cent. copper. | Grams copper. | Grams concentrate. | Per cent. copper. | Grams copper. | Recovery. | 80 |
|----------|------------|-------------------|---------------|--------------------|-------------------|---------------|-----------|----|
| F21.     | 750        | 2.01              | 15.07         | 45                 | 23.66             | 10.65         | 70.7%     |    |
| F22.     | 750        |                   |               | 47                 | 24.52             | 11.52         | 76.4%     |    |
| F27.     | 750        |                   |               | 43                 | 27.10             | 11.65         | 77.5%     |    |
| F28.     | 750        |                   |               | 47                 | 26.90             | 12.64         | 84.0%     |    |
| F45.     | 750        |                   |               | 51                 | 23.84             | 12.16         | 80.7%     |    |
| F46.     | 750        |                   |               | 48                 | 25.60             | 12.29         | 81.5%     |    |
| F47.     | 750        |                   |               | 27                 | 8.80              | 2.38          | 15.8%     |    |
| F48.     | 750        |                   |               | 28                 | 8.34              | 2.34          | 15.5%     |    |
| F49.     | 750        |                   |               | 62                 | 20.14             | 12.49         | 83.0%     |    |
| F50.     | 750        |                   |               | 63                 | 20.10             | 12.66         | 84.0%     |    |
| F51.     | 750        |                   |               | 60                 | 18.82             | 11.29         | 75.0%     |    |
| F52.     | 750        |                   |               | 62                 | 19.54             | 12.11         | 80.5%     |    |
| F53.     | 750        |                   |               | 29                 | 6.16              | 1.79          | 11.9%     |    |
| F54.     | 750        |                   |               | 30                 | 7.96              | 2.39          | 15.9%     |    |
| F55.     | 750        |                   |               | 59                 | 21.08             | 12.44         | 82.7%     |    |
| F56.     | 750        |                   |               | 56                 | 25.80             | 14.45         | 96.0%     |    |
| F64.     | 750        |                   |               | 65                 | 19.52             | 12.69         | 81.9%     |    |
| L27.     | 750        | 1.10              | 12.75         | 37                 | 28.42             | 10.51         | 81.7%     |    |
| L28.     | 750        | 1.10              | 12.75         | 34                 | 28.98             | 9.85          | 78.3%     |    |
| L29.     | 750        | 1.10              | 12.75         | 76                 | 5.66              | 4.30          | 33.4%     |    |
| L30.     | 750        | 1.10              | 12.75         | 83                 | 5.06              | 4.20          | 32.9%     |    |

95

Referring to the above table, tests marked F21, F22, F45, F46, F55, F56, were carried out with the addition to the 750 grams of ore of 10 grams of iron filings. In tests F27 and F28, two grams of iron filings were added. Tests F49 and F50 received ten grams of miscellaneous iron filings from the machine shop, and tests F51 and F52 received the same addition, the latter tests being made

100

however by a different observer. Tests F47, F48, F53, and F54 were blanks, in which only the regular oils and flotation media were used, no iron being added.

5 Test F64 was made with the same refractory ore, but instead of grinding it in a mill filled with flint pebbles, it was ground in a mill filled with steel balls, whereby particles of iron were introduced.

10 Tests L27 and L28 are blank tests on a good flotation ore, only the ordinary flotation oils being added. Tests L29 and L30 were made under identical conditions, except for the addition of 10 grams zinc filings.

15 It will be observed that with these particular ores, the efficiency of the process was entirely dependent upon the addition of iron.

20 The reasons underlying this observed effect are not as yet certainly known.

20 It is probable that the surface condition of the iron exercises an important influence. This is indicated by the fact which I have observed, that the addition of minute quantities of platinic chlorid to the solution materially increases the quantity of foam formed when air is blown through a porous diaphragm into a suspension or solution of a frothing agent in water, to which finely-divided iron has been added. In this case it is assumed that a small percentage of the iron is superficially replaced by platinum.

Instead of mixing iron filings with the ore favorable results are obtained by introducing finely-divided iron during the grinding or 35 reduction process. For example, test F64 in the foregoing tabular statement illustrates the effect of using steel balls in the grinding mill instead of the flint pebbles usually employed for the final reduction of the ore. In 40 this case iron in minute subdivision is thoroughly incorporated with the ore, owing to the abrasive effect of the latter upon the balls; and although this iron largely undergoes oxidation during and after the grinding 45 by the action of the air and water, it is found that a certain portion of it persists as metal, and tests have shown that the observed favorable action upon the flotation is due to this residual metal and not to the iron oxid 50 or hydroxid which accompanies it. When desired, the proportion of iron thus introduced may be increased by the use of balls of softer iron or steel, by the addition to the ore of some more highly abrasive material, by the 55 introduction of iron from other sources, or by a combination of such methods.

60 Not all forms of finely-divided iron are equally effective: for example, when sponge iron was substituted for the iron filings, equally favorable results were not secured.

Furthermore, certain solid materials have been shown to exert a distinctly unfavorable effect upon the flotation process. For example, referring to the foregoing tabular

statement (tests L27 to L30, inclusive), it 65 will be noted that the addition of a small proportion of zinc filings very markedly decreased the flotation efficiency in the case of a normally good flotation ore.

It is obviously impossible to name all of 70 the substances which may ultimately prove available for increasing the flotation efficiency, although the availability of any given substance is readily determined by simple experiment in the light of the information 75 herein given. Nor is it possible at the present time to define such available substances by a classification based upon other chemical 80 or physical properties which they may possess. Nevertheless, my invention is not restricted to the use of iron, but includes materials which are equivalent thereto in that they act to increase the efficiency of the flotation.

When the activating agent or substance is 85 to be used repeatedly, it is separated from the flotation tailings by known methods, depending upon its nature. Iron for example is easily recovered by magnetic separation; heavy substances may be recovered by concentrating tables; coarse substances by screening, etc. Classifiers may also be advantageously used for accomplishing a separation of the kind described. Combinations of 90 machines of various types may be employed. 95 For instance, where concentrating tables are used for re-treating flotation tailings, metallic iron will largely go into the table concentrates, and may by means of magnets and conveyer belts, be transferred again to the 100 flotation machine.

Although so far as is now known, the substances to be used as additions to the ore in accordance with this invention are active only in solid form, it is to be understood that 105 they may be introduced in solution, chemical reactions being relied upon to precipitate them in the active solid form, as in the example of platinic chlorid above referred to.

The present process is quite independent 110 of special apparatus, and may be carried out in any of the standard forms of flotation machines now on the market. The ore is either ground with the flotation agent, or is subsequently agitated therewith. The air 115 bubbles may be introduced as desired by any of the known methods, such as application of a vacuum, injection through a porous bottom, or by drawing or blowing air into the pulp and distributing it therethrough in 120 the form of small bubbles by violent agitation.

I claim:—

1. A process of concentrating ores by bubble-flotation, which consists in mixing 125 the ore with an extraneous solid capable of increasing the efficiency of the flotation, concentrating the mixture by flotation, recover-

ing the said extraneous solid from the flotation tailings, and applying the recovered solid in the flotation of other bodies of ore.

2. A process of concentrating ores by bubble-flotation, which consists in mixing iron in suitably subdivided form with the

ore, concentrating the mixture by flotation, recovering the metallic iron from the flotation tailings, and applying the recovered iron in the flotation of further bodies of ore. 10

In testimony whereof I affix my signature.

RUDOLF GAHL.